



US008819866B2

(12) **United States Patent**  
**Underwood et al.**

(10) **Patent No.:** **US 8,819,866 B2**  
(b5) **Date of Patent:** **Sep. 2, 2014**

- (54) **FLAME RESISTANT FABRIC AND GARMENTS MADE THEREFROM**
- (75) Inventors: **Joey K. Underwood**, Greenville, SC (US); **Jacques A. Cantin**, Greenville, SC (US); **Guy Connors Lucas**, Charlotte, NC (US)
- (73) Assignee: **International Textile Group, Inc.**, Greensboro, NC (US)
- (\*) Notice: Subject to any disclaimer, the term of this patent is extended or adjusted under 35 U.S.C. 154(b) by 19 days.

(21) Appl. No.: **13/436,081**

(22) Filed: **Mar. 30, 2012**

(65) **Prior Publication Data**

US 2013/0254980 A1 Oct. 3, 2013

- (51) **Int. Cl.**  
*A62B 17/00* (2006.01)  
*A41D 27/02* (2006.01)  
*A62B 5/00* (2006.01)

- (52) **U.S. Cl.**  
USPC ..... **2/81**; 2/69; 442/189; 139/420 A

- (58) **Field of Classification Search**  
None  
See application file for complete search history.

(56) **References Cited**

U.S. PATENT DOCUMENTS

- 3,729,920 A 5/1973 Sayers et al.  
4,304,811 A 12/1981 David et al.  
4,749,378 A \* 6/1988 Cates et al. ..... 8/130.1  
4,759,770 A \* 7/1988 Cates et al. ..... 8/490  
5,299,602 A 4/1994 Barbeau et al.  
5,858,888 A \* 1/1999 Underwood et al. ..... 442/286  
5,928,971 A 7/1999 Ellis et al.

- 6,065,153 A \* 5/2000 Underwood et al. ..... 2/93  
6,132,476 A \* 10/2000 Lunsford et al. ..... 8/531  
6,192,520 B1 \* 2/2001 Underwood et al. ..... 2/93  
6,247,179 B1 \* 6/2001 Underwood et al. ..... 2/81  
6,460,321 B1 10/2002 Koshimae et al.  
6,547,835 B1 \* 4/2003 Lunsford et al. ..... 8/531  
6,606,749 B2 \* 8/2003 Underwood et al. ..... 2/93  
6,624,096 B2 \* 9/2003 Thomas et al. ..... 442/181  
6,818,024 B2 \* 11/2004 Lunsford et al. ..... 8/531  
6,867,154 B1 \* 3/2005 Lunsford et al. ..... 442/136  
6,886,184 B2 \* 5/2005 Underwood et al. ..... 2/82  
7,393,800 B2 7/2008 Corner  
7,581,260 B2 \* 9/2009 Underwood et al. ..... 2/82  
7,589,036 B2 9/2009 Corner et al.  
7,811,952 B2 \* 10/2010 Truesdale et al. ..... 442/131

(Continued)

FOREIGN PATENT DOCUMENTS

- GB 2275934 9/1994  
WO WO 2011/050376 A1 5/2011

OTHER PUBLICATIONS

Duralite Fabric Information Including Morning Pride Press Release and Slides, 7 pages.  
Safety Conappnents Data Sheet on ARMOR 5.5, one page.

(Continued)

*Primary Examiner* — Bobby Muromoto, Jr.

(74) *Attorney, Agent, or Firm* — Dority & Manning, P.A.

(57) **ABSTRACT**

Protective garments include a flame resistant fabric that is strong and yet has a soft hand. The fabric is made from a combination of filament yarns and spun yarns. The filament yarns and spun yarns are woven together such that the filament yarns are separated by from about 2 to about 5 spun yarns in both the warp direction and the fill direction. The spun yarns may contain polybenzimidazole fibers in combination with other fibers, such as aramid fibers. The filament yarns may comprise para-aramid fibers. In one embodiment, the filament yarns may have a size larger than the spun yarns.

**22 Claims, 8 Drawing Sheets**



(56)

**References Cited****U.S. PATENT DOCUMENTS**

7,862,865 B2 1/2011 Truesdale, III et al.  
8,071,492 B2 \* 12/2011 Hess et al. .... 442/302  
8,209,785 B2 \* 7/2012 Underwood et al. .... 2/458  
2002/0026663 A1 \* 3/2002 Underwood et al. .... 2/458  
2002/0106955 A1 \* 8/2002 Underwood et al. .... 442/148  
2003/0040240 A1 2/2003 Thomas  
2003/0203690 A1 10/2003 Hess et al.  
2003/0228812 A1 12/2003 Stanhope et al.  
2004/0034905 A1 \* 2/2004 Underwood et al. .... 2/458  
2004/0092187 A1 5/2004 Favier et al.  
2004/0152378 A1 8/2004 Stanhope et al.  
2005/0155131 A1 \* 7/2005 Underwood et al. .... 2/85

2005/0158559 A1 \* 7/2005 Martin et al. .... 428/422  
2006/0154542 A1 \* 7/2006 Underwood et al. .... 442/82  
2007/0072502 A1 \* 3/2007 Underwood et al. .... 442/82  
2011/0165807 A1 \* 7/2011 Underwood et al. .... 442/76  
2011/0191949 A1 \* 8/2011 Underwood et al. .... 2/458  
2012/0270456 A1 10/2012 Gstettner et al.  
2012/0278979 A1 \* 11/2012 Underwood et al. .... 2/455

**OTHER PUBLICATIONS**

Safety Components Brochure on ARMOR 7.0, 34 pages.  
Extended European Search Report for EP Application No. 12167962.  
5-2314, dated Dec. 12, 2012.

\* cited by examiner



*FIG. -1-*



*FIG. -2-*



*FIG. -3-*



*FIG. -4-*



*FIG. -5-*



*FIG. -6-*



*FIG. -7-*



*FIG. -8-*

## FLAME RESISTANT FABRIC AND GARMENTS MADE THEREFROM

## BACKGROUND

Various different types of protective garments exist that are intended to provide protection to the wearer. In certain embodiments, for instance, the protective garments are designed to provide protection from heat and flame so as to prevent burn injuries. Such protective garments, for instance, are typically worn by firefighters, other service providers, and military personnel. Military personnel, for instance, wear such garments to provide protection against incendiary devices and the like.

Such garments should be fire resistant while also being as light as possible, strong, abrasion resistant, rip and tear resistant, flexible, and should encumber the wearer as little as possible.

Conventional firefighter garments, for instance, are generally constructed having a number of discrete layers. Typically, these layers include an outer shell, a moisture barrier layer, a thermal barrier layer, and an inner lining. The layers are generally made from appropriate thermally-resistant materials to provide protection against heat and flame.

Protective garments for firefighters that are also water resistant are disclosed in U.S. Pat. No. 7,581,260, which is incorporated herein by reference. The '260 patent discloses various garments and fabrics that have made great advances in the art.

Improvements, however, are still needed in designing fabrics for protective garments that are intended to provide fire resistance. In particular, a need exists for lighter fabrics that provide the same or better physical properties than current commercial products. A need also exists for a fabric that has a soft hand, meaning that the fabric is flexible and easy to maneuver in when worn.

## SUMMARY

In general, the present disclosure is directed to flame resistant garments that are made from a flame resistant fabric. The flame resistant garment, for instance, may comprise any protective garment designed to protect a wearer from exposure to heat and/or flame. In one embodiment, for instance, the protective garment may comprise a fireman turnout coat, trousers worn by firemen, or any other garment worn by firefighters. In an alternative embodiment, the garment may comprise apparel worn by military personnel. For instance, the garment may comprise a bomb suit, tank uniform, other combat garments, a flight jacket, or the like. In still another embodiment, the garment may comprise industrial workwear or may comprise a protective chemical suit. The garment may comprise a shirt, a coat, a jacket, trousers, gloves, boots, protective headgear such as a hat, or the like.

In one embodiment, the present disclosure is directed to a flame resistant garment that includes a fabric shaped to cover at least a portion of a wearer's body. The fabric comprises first yarns combined with second yarns. The first yarns comprise filament yarns comprised of an inherently flame resistant material. For instance, the filament yarns may be made from an aramid polymer, such as a para-aramid polymer or a meta-aramid polymer. The second yarns, on the other hand, comprise spun yarns which may contain fibers comprised of polybenzimidazole and fibers comprised of an aramid polymer. In accordance with the present disclosure, the first yarns and the second yarns are contained in the fabric in a ratio of from about 1:1 to about 1:5, such as greater than 1:1 to about 1:5.

For instance, in one embodiment, the first and second yarns are contained in the fabric in a ratio of 1:2 such that for every filament yarn there are two spun yarns.

The fabric described above, for instance, may have a warp direction and a fill direction. The ratio between the first yarn and the second yarn can be the same in both the warp and fill direction or may be different between the warp and fill directions. In one particular embodiment, for instance, the ratio of the first yarns to the second yarns in the warp direction and the fill direction is 1:2.

10 In one embodiment, the spun yarn can contain polybenzimidazole fibers in an amount from about 30% to about 60% by weight, such as in an amount from about 40% to about 55% by weight. The entire fabric, for instance, may contain polybenzimidazole fibers in an amount of at least about 20% by weight, such as in an amount of at least about 25% by weight, such as in an amount of at least about 30% by weight, such as in an amount of at least about 35% by weight, such as in an amount of at least about 40% by weight. Polybenzimidazole fibers are contained in the fabric in an amount generally less than about 70% by weight, such as in an amount less than about 60% by weight, such as in an amount less than about 50% by weight.

15 The fabric can have any suitable weave depending on the particular application and desired result. For instance, the fabric may have a rip stop weave, a herringbone weave, or a plain weave. In one embodiment, the fabric may have a twill weave.

20 In one embodiment, the filament yarns can optionally have a bigger size than the spun yarns. As used herein, the size of a yarn refers to its weight per unit length. Thus, when the filament yarns have a denier of 600, the spun yarns have a size of 18/2 or less. When the filament yarns have a denier of 400, on the other hand, the spun yarns can have a size of 27/2 or less. When the filament yarns have a denier of 200, the spun yarns can have a size of 54/2 or less. In general, the spun yarns have a size of 108/2 or greater, such as greater than 70/2 or greater than 60/2.

25 Of particular advantage, fabrics made according to the present disclosure can have excellent physical properties at relatively light weights. The fabric, for instance, may have a basis weight of less than about 8 osy, such as less than about 7.5 osy, such as less than about 7 osy, such as less than about 6.5 osy, such as less than about 6.0 osy. The basis weight of the fabric is generally greater than about 3 osy, such as greater than about 4 osy, such as greater than about 4.5 osy. In certain embodiments, the basis weight is from about 5.5 osy to about 6.5 osy or from about 6.0 osy to about 7.5 osy. Within the above weight ranges, the fabric can have a circular bend in the warp direction or in the fill direction of from about 2 lbs. to about 5 lbs. when tested according to ASTM Test D4032. The fabric can have a break strength in the fill direction of from about 400 lbs. to about 800 lbs. when tested according to ASTM Test D5034. The fabric can have a trap tear in the warp direction of from about 300 lbs. to about 450 lbs. and can have a trap tear in the fill direction of from about 250 lbs. to about 400 lbs. when tested according to ASTM Test D5587.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410

forth more particularly in the remainder of the specification, including reference to the accompanying figures, in which:

FIG. 1 is a perspective view of one embodiment of a protective garment made in accordance with the present disclosure;

FIG. 2 is a cross-sectional view of the garment illustrated in FIG. 1;

FIG. 3 is a perspective view of one embodiment of trousers made in accordance with the present disclosure;

FIG. 4 is a front perspective view of a first embodiment of a coat showing a design as embodied by a fabric used to construct the coat;

FIG. 5 is a front perspective view of a first embodiment of trousers showing the design illustrated in FIG. 4;

FIG. 6 is a plan view of one side of a fabric that embodies the design as illustrated in FIGS. 4 and 5;

FIG. 7 is a plan view of an opposite side of a fabric that embodies the design illustrated in FIGS. 4 and 5; and

FIG. 8 is a plan view of an opposite side of the fabric that embodies the design illustrated in FIGS. 4 and 5.

Repeat use of reference characters in the present specification and drawings is intended to represent the same or analogous features or elements of the present invention.

#### DETAILED DESCRIPTION

It is to be understood by one of ordinary skill in the art that the present discussion is a description of exemplary embodiments only, and is not intended as limiting the broader aspects of the present disclosure.

In general, the present disclosure is directed to protective garments that provide heat and flame resistance to a wearer. In accordance with the present disclosure, the protective garments are made from a flame resistant fabric. The fabric includes a combination of filament yarns and spun yarns that are each primarily made from inherently flame resistant materials. The spun yarns contain polybenzimidazole fibers that enhance the flame resistant properties of the fabric.

As will be described in greater detail below, the filament yarns and the spun yarns are woven together in a manner that produces a fabric with excellent physical properties. For instance, the fabric has excellent strength properties in combination with excellent tactile qualities. In particular, the fabric is very strong while also having a soft hand and being very flexible. Of particular advantage, the above characteristics and properties are obtained at relatively low fabric weights. Consequently, garments made from the above described fabric not only provide excellent thermal protection, but are also very comfortable to wear.

Various protective garments may be made in accordance with the present disclosure. The protective garments include, for instance, footwear, trousers, jackets, coats, shirts, headwear, gloves, and the like. The fabric can also be used to construct one-piece jumpsuits, which may be well suited for use in industrial settings.

The garments can be constructed so as to be worn in all types of environments and can be worn by people with different occupations. In one embodiment, the garment may comprise a military garment, such as a battledress uniform. The garment may also comprise various other military apparel, such as flight suits, military jackets, military parkas, and the like.

In one embodiment, the fabric may be used to construct a garment worn by firefighters. For instance, referring to FIG. 1, one embodiment of a fireman turnout coat 10 constructed in accordance with the present disclosure is illustrated. Garment 10 includes a relatively tough outer shell 12 having a liner

assembly 14 located therein. Outer shell 12 and liner assembly 14 together function to protect a wearer from heat and flame such as may be encountered during firefighting activities.

5 In the illustrated embodiment, liner assembly 14 is constructed as a separate unit that may be removed from outer shell 12. A zipper 16 is provided for removably securing liner assembly 14 to outer shell 12. It should be appreciated, however, that other suitable means of attachment, including a more permanent type of attachment such as stitches, may also be used between liner assembly 14 and outer shell 12.

The construction of protective garment 10 is more particularly illustrated in FIG. 2. As shown, liner assembly 14 includes a plurality of material layers quilted together. The outermost layers, i.e. lining layers 20 and 22, are connected together about their respective peripheries to form an inner cavity. A thermal barrier layer 24 and a moisture barrier layer 26 are located within the inner cavity, as shown. Typically, lining layer 20 will be adjacent the wearer's body during use, whereas lining layer 22 will be adjacent outer shell 12.

Thermal barrier layer 24 can be made from various materials. For instance, an aramid felt, such as a felt produced from NOMEX fibers obtained from DuPont can be used. The felt functions as an insulator to inhibit transfer of heat from the ambient-environment to the wearer.

25 Moisture barrier 26 is preferably a suitable polymeric membrane that is impermeable to liquid water but is permeable to water vapor. Moisture barrier layer 26 is designed to prevent water contacting the exterior surface of garment 10 from reaching the wearer while at the same time permitting the escape of perspiration from the wearer.

In the embodiment described above, the fireman turnout coat 10 includes multiple layers. In other embodiments, however, it should be understood that a coat or jacket made in accordance with the present disclosure may include a single layer or may include an outer shell attached to a liner. For example, wildland firefighter garments are typically one or two layers.

30 Referring to FIG. 3, a pair of trousers made in accordance with the present disclosure is shown. The trousers 40 as shown in FIG. 3 can be used in conjunction with the turnout coat 10 illustrated in FIG. 1. The trousers 40 also include an outer shell 12 made from the fabric of the present disclosure.

In accordance with the present disclosure, the outer shell 45 12 is made from a fabric containing filament yarns and spun yarns. The filament yarns and spun yarns are made from fire resistant materials, such as inherently flame resistant fibers. As will be described in greater detail below, the spun yarns and filament yarns are constructed from materials and woven together in a manner that produces a fabric having excellent thermal and physical properties at relatively low basis weights. Of particular advantage, the fabric also has a soft hand, meaning that the fabric is flexible and therefore comfortable to wear.

55 In one embodiment, for instance, the fabric used to produce the outer shell 12 of the garment 10 may include a plurality of warp yarns interwoven with a plurality of fill yarns. In accordance with the present disclosure, at least certain of the warp yarns are filament yarns and at least certain of the fill yarns are filament yarns. The remaining yarns in the fabric, on the other hand, may comprise spun yarns.

In one embodiment, the filament yarns may be made from an inherently flame resistant material. For example, the filament yarns may be made from an aramid filament, such as a para-aramid filament. The use of a para-aramid filament yarn increases the strength of the fabric while also providing excellent flame resistant properties.

## 5

In other embodiments, the filament yarns may be made from other flame resistant materials. For instance, the filament yarns may be made from poly-p-phenylenebenzobisoxazole fibers (PBO fibers), and/or FR cellulose fibers, such as FR viscose filament fibers.

The filament yarns are combined with spun yarns. In accordance with the present disclosure, the spun yarns, in one embodiment, may contain polybenzimidazole fibers alone or in combination with other fibers. For example, in one embodiment, the spun yarns may contain polybenzimidazole fibers in combination with aramid fibers, such as para-aramid fibers, meta-aramid fibers, or mixtures thereof.

Instead of or in addition to containing polybenzimidazole fibers, the spun yarns may contain aramid fibers as described above, modacrylic fibers, preoxidized carbon fibers, melamine fibers, polyamide imide fibers, polyimide fibers, and mixtures thereof.

In one particular embodiment, the spun yarns contain polybenzimidazole fibers in an amount greater than about 30% by weight, such as in an amount greater than about 40% by weight. The polybenzimidazole fibers may be present in the spun yarns in an amount less than about 60% by weight, such as in an amount less than about 55% by weight. The remainder of the fibers, on the other hand, may comprise para-aramid fibers.

In one embodiment, various other fibers may be present in the spun yarns. When the fabric is used to produce turnout coats for firemen, the spun yarns can be made exclusively from inherently flame resistant fibers. When the fabric is being used in other applications, however, various other fibers may be present in the spun yarns. For instance, the spun yarns may contain fibers treated with a fire retardant, such as FR cellulose fibers. Such fibers can include FR cotton, FR rayon, FR acetate, FR triacetate, and FR lyocell, and the like. The spun yarns may also contain nylon fibers if desired, such as antistatic fibers.

In accordance with the present disclosure, the filament yarns and the spun yarns are woven together such that the ratio of filament yarns to spun yarns can be from about 1:1 to about 1:5, such as greater than 1:1 to about 1:4. In one embodiment, for instance, the ratio between the filament yarns and the spun yarns can be from about 2:3 to about 1:3. In one particular embodiment, the fabric contains two spun yarns for each filament yarn.

Woven fabrics made in accordance with the present disclosure generally include a warp direction and a fill direction. The ratio of filament yarns to spun yarns in each direction of the fabric can be the same or different. For example, in one embodiment, a greater density of filament yarns may be present in the warp direction than the fill direction or a greater density of filament yarns may be present in the fill direction than the warp direction. In one embodiment, the spun yarns and filament yarns are present in the fabric such that the fabric contains polybenzimidazole fibers in an amount of at least about 20% by weight, such as in an amount of at least about 25% by weight, such as in an amount of at least about 30% by weight, such as in an amount of at least about 35% by weight, such as in an amount of at least about 40% by weight. In general, the polybenzimidazole fibers may be present in the fabric in an overall amount of less than about 70% by weight, such as less than about 60% by weight, such as less than about 50% by weight.

In general, various different weave patterns may be used to produce the fabric. For instance, a twill weave, a plain weave, a rip stop weave, or a herringbone weave may be used. In one particular embodiment, the fabric may have a twill weave. The twill weave may have a 2x1 or a 3x1 weave. In a twill

## 6

weave, crossings of adjacent warps occur along diagonal twill lines. In a 2x1 twill weave, the warp yarns pass over two fill yarns before interlacing with a third yarn. The interfacing are offset along a diagonal to produce characteristic twill lines.

5 The sizes of the yarns and the basis weight of the fabric can vary depending upon the particular application and the desired results. As used herein, the size of a yarn refers to its weight per unit length. For filament yarns, size is measured in denier, while for spun yarns size is measured as yarn count. As 10 used herein, a larger sized yarn is generally coarser while a smaller sized yarn is finer. In general, the filament yarns can have a denier of greater than about 100, such as greater than about 200. The denier is generally less than about 1000, such as less than about 900. The spun yarn, on the other hand, can have a count or size of generally greater (more coarse) than about 108/2, such as greater than 70/2 and can have a count of less than (finer) about 14/2, such as less than about 18/2.

In one embodiment, the size of the filament yarns may be greater than the size of the spun yarns. In fact, various advantages and benefits may be obtained by having the size of the filament yarn larger than the size of the spun yarn. Increasing the size of the filament yarn, for instance, may dramatically increase the strength of the fabric. The manner in which the yarns are woven together, however, prevents the filament 20 25 yarns from creating issues with snagging or abrasion resistance.

For example, when the filament yarns have a denier of 800, the spun yarns can have a size or count of 14/2 or finer. When the filament yarns have a denier of 600, the spun yarns can 30 have a count of 18/2 or finer, such as 20/2 or finer. When the filament yarns have a denier of 400, the spun yarns can have a count of about 27/2 or finer, such as about 32/2 or finer. When the filament yarns have a denier of 200, on the other hand, the spun yarns can have a count of about 54/2 or finer. 35 When the filament yarns have a denier of about 100, the spun yarns can have a count of about 108/2 or finer.

In one embodiment, the filament yarns can have a denier of from about 200 to 600, while the spun yarns can have a count of from about 54/2 to about 14/2.

40 Although various benefits may be obtained by having the size of the filament yarn be larger than the size of the spun yarn, in other embodiments, there may be advantages to having the spun yarn be larger in size than the filament yarn.

The basis weight of fabrics made according to the present 45 disclosure can vary depending upon various factors and the end use application. Of particular advantage, fabrics made according to the present disclosure can have excellent properties at relatively lighter basis weights. In general, the fabric can have a basis weight of from about 2 osy to about 9 osy, such as from about 4 osy to about 8 osy. In one embodiment, the basis weight can be less than about 7 osy, such as less than about 7.5 osy. In particular, it was discovered that fabrics made according to the present disclosure can have a basis weight of from about 6 osy to about 6.9 osy, while still having 50 55 many of the physical properties of conventional fabrics having a basis weight of about 7.5 osy or greater.

Once the fabric is constructed, the fabric may be treated with various coatings and finishes as may be desired. In one embodiment, for instance, the fabric may be treated with a durable water resistant treatment. The durable water resistant treatment may comprise, for instance, a fluoropolymer. Other treatments that may be applied to the fabric include insect repellants and/or a moisture management finish.

Many different types of durable water resistant treatments 60 65 may be applied to the fabric. In one embodiment, the durable water resistant treatment forms a finish (as opposed to a coating) on the fabric. The durable water resistant treatment

can be applied to the fabric by treating the fabric with a bath containing the treatment, padding the composition into the fabric, placing the fabric on a tenter frame, and heating the fabric in order to evaporate all volatiles. During the process, the durable water resistant treatment may be applied to the fabric in an amount from about 0.5% to about 10% by weight, such as from about 1% to about 5% by weight.

In many applications, the durable water resistant treatment may comprise a fluoropolymer. Particular durable water resistant treatments that may be applied to the fabric in accordance with the present disclosure are discussed in greater detail below.

In one embodiment, the DWR comprises at least one member selected from the group consisting of a perfluoroalkyl group-containing substance, a fluorine-containing surfactant, a fluorine-containing oil, a fluorosilicone oil and a silicone oil. Preferably the fluorine-containing resin derives from an aqueous dispersion or dissolving in a solvent. Preferably, the fluorine-containing resin comprises a fluororesin or a mixture of a fluororesin and some other resin. Preferably, the fluororesin is a copolymer of a fluoroolefin and a vinyl monomer. Preferably, the fluororesin is a copolymer of fluoroolefins. Preferably, the copolymer of fluoroolefins is a copolymer of vinylidene fluoride and a fluoroolefin other than vinylidene fluoride.

In another embodiment, a durable water/soil-resistant fluoropolymer is selected from those groups that will provide the necessary water/soil resistance and can be polymerized. Examples include fluorinated monomers of acrylates, methacrylates, alkenes, alkenyl ethers, styrenes, and the like. Monomers that contain carbon-fluorine bonds that are useful include, but are not limited to, Zonyl TA-N (an acrylate from DuPont), Zonyl<sup>TM</sup> (a methacrylate from DuPont), FX-13 (an acrylate from 3M), and FX-14 (a methacrylate from 3M) or UNIDYNE TG581 (a C<sub>6</sub> fluoropolymer available from Daikin). The fluoropolymers may include —CF<sub>3</sub> and —CHF<sub>2</sub> end groups, perfluoroisopropoxy groups (—OCF(CF<sub>3</sub>)<sub>2</sub>), 3,3,3-trifluoropropyl groups, and the like. The polymers may include vinyl ethers having perfluorinated or partially fluorinated alkyl chains. The fluoropolymer preferably comprises one or more fluoroaliphatic radical-containing monomers. Monomers used to form the fluoropolymer may be based upon 6 carbon chain chemistry or 8 carbon chain chemistry.

In another embodiment, the DWR comprises a repellent and a fluorine-containing resin, wherein the repellent comprises an esterification reaction product (I-3) from a perfluoroalkyl group-containing compound (I-3-1) and a compound (I-3-2) containing a phosphoric acid group as a functional group, and the fluorine-containing resin derives from an aqueous dispersion. Preferably, the fluorine-containing resin comprises a fluororesin or a mixture of a fluororesin and some other resin. Preferably, the other resin is an acrylic resin. Preferably, the fluororesin is a copolymer of a fluoroolefin and a vinyl monomer. Preferably, the fluororesin is a copolymer of fluoroolefins. Preferably, the copolymer of fluoroolefins is a copolymer of vinylidene fluoride and a fluoroolefin other than vinylidene fluoride. Preferably, the fluorine-containing resin comprises a fluororesin obtained by seed polymerization of an acrylic resin.

Commercially available DWR not mentioned above that may be used in the present disclosure include fluoropolymer compositions sold under the name MILEASE<sup>®</sup> by Clariant, fluorochemicals sold under the tradename TEFILON<sup>®</sup> or Capstone<sup>®</sup> by DuPont, fluorochemicals sold under the tradename ZEPEL<sup>®</sup> also by DuPont, or fluorocarbon polymers sold under the tradename REPEARL<sup>®</sup> by the Mitsubishi

ishi Chemical Company or fluorocarbon polymers sold under the tradename UNIDYNE<sup>®</sup> by the Daikin Company.

In one embodiment, if desired, an isocyanate may be present in conjunction with a fluorochemical, such as a fluoropolymer. The isocyanate may comprise a blocked isocyanate that is a formaldehyde-free cross-linking agent for fluorochemical finishes. The blocking agent may comprise a phenol or any other suitable constituent.

Once treated with a durable water resistant treatment, the fabric may have a spray rating of at least 70, such as at least 80, such as even greater than 90 after 5 laundry cycles, after 10 laundry cycles, after 20 laundry cycles, and even after 30 laundry cycles. The spray rating of a fabric is determined according to AATCC 22 and is described in U.S. Pat. No. 7,581,260.

15 Fabrics made according to the present disclosure can have excellent tensile strength properties. For instance, the fabric can have a break strength according to ASTM D5034 in the fill direction of greater than about 400 lbs., such as greater than about 450 lbs., such as greater than about 550 lbs., such as greater than about 600 lbs., such as greater than about 620 lbs. at a fabric weight of from about 5 osy to about 8 osy, and particularly from about 7 osy to about 7.5 osy. The break strength in the warp direction can generally be greater than about 400 lbs., such as greater than about 500 lbs., such as greater than about 550 lbs. The break strength is generally less than about 800 lbs.

20 The fabric can display a trap tear according to ASTM Test D5587 of greater than about 200 lbs., such as greater than about 250 lbs., such as greater than about 275 lbs., such as greater than about 290 lbs. in the fill direction. In the warp direction, the trap tear can be generally greater than about 200 lbs., such as greater than about 250 lbs., such as greater than about 300 lbs., such as greater than about 325 lbs., such as greater than about 335 lbs. The trap tear in the fill direction and in the warp direction is generally less than about 500 lbs. at the basis weights described above with respect to the break strength.

25 The fabric can have the above strength properties while being very flexible. For instance, when tested according to the 30 circular bend test according to ASTM Test D4032, the fabric can have a circular bend in the fill direction of less than about 6 lbs., such as less than about 5.5 lbs., such as less than about 5 lbs., such as even less than about 4.5 lbs., especially for a fabric having a weight of from about 6.5 osy to about 7 osy. In the warp direction, the circular bend can generally be less than about 5 lbs., such as less than about 4.5 lbs., such as less than about 4 lbs., such as even less than about 3.5 lbs. In general, the circular bend is greater than about 1 lb. in both the fill direction and warp direction.

35 On a weight basis, fabrics made according to the present invention can have a break strength in the fill direction or in the warp direction of greater than about 60 lbs. per osy, such as greater than about 65 lbs. per osy, such as greater than about 70 lbs. per osy, such as greater than about 75 lbs. per osy, such as even greater than about 80 lbs. per osy. The break strength per weight is generally less than about 120 lbs. per osy. The trap tear in the fill direction or the warp direction can generally be greater than about 40 lbs. per osy, such as greater than about 42 lbs. per osy, such as greater than about 46 lbs. per osy. The trap tear per weight is generally less than about 70 lbs. per osy.

40 The fabric of the present disclosure also possesses excellent thermal properties. For instance, when tested according to ASTM Test D6413, the fabric can have a char length in both the fill and warp direction of less than about 10 mm, such as less than about 9 mm, such as even less than about 8 mm. The char length is generally greater than about 1 mm.

In addition to having excellent mechanical properties and fire resistant properties, fabrics made in accordance with the present disclosure may also display a new, original and ornamental design. For instance, one embodiment of a design in accordance with the present disclosure is illustrated in FIGS. 4-8.

The present disclosure may be better understood with reference to the following examples.

Example No. 1

The following fabrics were produced and tested for various properties. Sample Nos. 1 and 2 described below represent previously made fabrics including a grid-like pattern. Sample Nos. 3 and 4, on the other hand, were made in accordance with the present disclosure. As shown below, a fabric made in accordance with the present disclosure demonstrated not only excellent strength characteristics and flexibility characteristics but also possessed excellent flame resistance.

Sample No. 1

This fabric contained spun yarns and filament yarns in a plain weave. The filament yarns formed a grid-like pattern in the fabric.

Warp Yarn: 21/2 Spun yarn containing 40% polybenzimidazole fibers and 60% para-aramid fibers. The second warp yarn was a 600 denier multi-filament yarn containing para-aramid fibers. The filament yarn accounted for every tenth yarn in the warp direction.

Fill Yarn: 21/2 Spun yarn containing 40% polybenzimidazole fibers and 60% para-aramid fibers. The second fill yarn was a 600 denier multi-filament yarn containing para-aramid fibers. The filament yarn accounted for every tenth yarn in the fill direction.

Ends: 51 per inch

Picks: 51 per inch

Weight: 7.39 osy

Weave: Plain weave

Sample No. 2

This fabric contained spun yarns and filament yarns in a plain weave. The filament yarns formed a grid-like pattern in the fabric.

Warp Yarn: 21/2 Spun yarn containing 40% polybenzimidazole fibers and 60% para-aramid fibers. The second warp yarn was a 600 denier multi-filament yarn containing para-aramid fibers. The filament yarn accounted for every seventh yarn in the warp direction.

Fill Yarn: 21/2 Spun yarn containing 40% polybenzimidazole fibers and 60% para-aramid fibers. The second fill yarn was a 600 denier multi-filament yarn containing para-aramid fibers. The filament yarn accounted for every seventh yarn in the fill direction.

Ends: 51 per inch

Picks: 51 per inch

Weight: 7.58 osy

Weave: Plain weave

Sample No. 3

The below fabric included spun yarns and filament yarns in both the warp direction and the fill direction. The weave pattern included two spun yarns, one filament yarn, two spun yarns, one filament yarn, etc. in both the fill direction and the warp direction.

Warp Yarn: 18/2 Spun yarn containing 61.6% para-aramid fibers and 38.4% meta-aramid fibers. The filament yarn was a 600 denier filament yarn containing para-aramid fibers.

Fill Yarn: 18/2 Spun yarn containing 61.6% para-aramid fibers and 38.4% meta-aramid fibers. The filament yarn was a 600 denier filament yarn containing para-aramid fibers.

Ends: 48 per inch

Picks: 42 per inch

Weight: 7.12 osy

Weave: 2x1 twill weave

Sample No. 4

The below fabric included spun yarns and filament yarns in both the warp direction and the fill direction. The weave pattern included two spun yarns, one filament yarn, two spun yarns, one filament yarn, etc. in both the fill direction and the warp direction.

Warp Yarn: 26/3 spun yarn containing 55% para-aramid fibers and 45% polybenzimidazole fibers. The filament yarn was a 600 denier filament yarn containing para-aramid fibers.

Fill Yarn: 26/3 spun yarn containing 55% para-aramid fibers and 45% polybenzimidazole fibers. The filament yarn was a 600 denier filament yarn containing para-aramid fibers.

Ends: 46 per inch

Picks: 41 per inch

Weight: 7.21 osy

Weave: 2x1 twill weave

Sample No. 5

The below fabric included spun yarns and filament yarns in both the warp direction and the fill direction. The weave pattern included two spun yarns, one filament yarn, two spun yarns, one filament yarn, etc. in both the fill direction and the warp direction.

Warp Yarn: 18/2 spun yarn containing 48% para-aramid fibers and 52% polybenzimidazole fibers. The filament yarn was a 600 denier filament yarn containing para-aramid fibers.

Fill Yarn: 18/2 spun yarn containing 48% para-aramid fibers and 52% polybenzimidazole fibers. The filament yarn was a 600 denier filament yarn containing para-aramid fibers.

Ends: 43 per inch

Picks: 43 per inch

Weight: 7.00 osy

Weave: 2x1 twill weave

| TEST__METHOD | TEST__NAME                       | UNIT                      | Sample 1 | Sample 2 | Sample 3 | Sample 4 | Sample 5 |
|--------------|----------------------------------|---------------------------|----------|----------|----------|----------|----------|
| AATCC 118    | OIL REPELLENCY                   | AATCC<br>SCALE            | 6        | 6        | 6        | 6        | 6        |
| AATCC 135    | SHRINK FILL 5X<br>SHRINK WARP 5X | PERCENT                   | 3.1      | 2.1      | 0.0      | 0.8      | 0.1      |
| AATCC 193    | WATER REPELLENCY                 | PERCENT<br>AATCC<br>SCALE | 1.7      | 1.0      | 2.8      | 2.0      | 0.2      |
| AATCC 22     | SPRAY RATING                     | AATCC<br>SCALE            | 100      | 100      | 100      | 100      | 100      |

-continued

| TEST_METHOD                  | TEST_NAME               | UNIT     | Sample 1 | Sample 2 | Sample 3 | Sample 4 | Sample 5 |
|------------------------------|-------------------------|----------|----------|----------|----------|----------|----------|
| AATCC 42                     | WATER ABSORPTION        | PERCENT  | 0.2      | 0.3      | 0.6      | 0.9      | 1.0      |
| AATCC 42<br>(AATCC 135)      | WATER ABSORPTION 5X     | PERCENT  | 0.8      | 0.4      | 0.0      | 1.6      | 1.8      |
| ASTM D 1777                  | THICKNESS               | INCHES   | 0.015    | 0.017    | 0.016    | 0.018    | 0.017    |
| ASTM D 3774                  | WIDTH                   | INCHES   | 61.15    | 61.01    | 61.25    | 60.25    | 61.00    |
| ASTM D 3775                  | ENDS                    | THRDS_IN | 51       | 51       | 49       | 46       | 43       |
|                              | PICKS                   | THRDS_IN | 52       | 50       | 45       | 40       | 43       |
| ASTM D 3776                  | WEIGHT                  | OZ_SQ_YD | 7.39     | 7.58     | 7.12     | 7.21     | 7.00     |
| ASTM D4032                   | CIRCULAR BEND FILL      | POUNDS   | 6.4      | 6.9      | 5.7      | 4.2      | 3.1      |
|                              | CIRCULAR BEND WARP      | POUNDS   | 6.1      | 6.0      | 5.4      | 3.3      | 3.1      |
| ASTM D 5034                  | BREAK STRENGTH FILL     | POUNDS   | 356      | 417      | 636      | 623      | 468      |
|                              | BREAK STRENGTH WARP     | POUNDS   | 275      | 335      | 615      | 588      | 456      |
| ASTM D 5034<br>(AATCC 135)   | BREAK STRENGTH FILL 5X  | POUNDS   | 296      | 335      | 529      | 552      | 498      |
| ASTM D 5587                  | BREAK STRENGTH WARP 5X  | POUNDS   | 252      | 282      | 592      | 521      | 466      |
| ASTM D 5587                  | TRAP TEAR FILL          | POUNDS   | 123      | 277      | 205      | 296      | 313      |
|                              | TRAP TEAR WARP          | POUNDS   | 121      | 167      | 282      | 341      | 219      |
| ASTM D 5587<br>(AATCC 135)   | TRAP TEAR FILL 5X       | POUNDS   | 70       | 113      |          | 231      | 218      |
|                              | TRAP TEAR WARP 5X       | POUNDS   | 90       | 109      |          | 322      | 213      |
| ASTM D 6413<br>(AATCC 135)   | AFTER FLAME FILL        | SECONDS  | 0        | 0        | 0        | 0        | 0        |
|                              | AFTER FLAME WARP        | SECONDS  | 0        | 0        | 0        | 0        | 0        |
|                              | AFTER GLOW FILL         | SECONDS  | 5        | 7        | 8        | 5        | 3        |
|                              | AFTER GLOW WARP         | SECONDS  | 5        | 7        | 8        | 5        | 4        |
|                              | CHAR LENGTH FILL        | MM       | 16       | 16       | 13       | 8        | 9        |
|                              | CHAR LENGTH WARP        | MM       | 15       | 16       | 12       | 6        | 10       |
|                              | DRIP FILL               | NONE     | 0        | 0        | 0        | 0        | 0        |
|                              | DRIP WARP               | NONE     | 0        | 0        | 0        | 0        | 0        |
| ASTM D 6413<br>(AATCC 135)   | AFTER FLAME FILL 5X     | SECONDS  | 0        | 0        | 0        | 0        | 0        |
|                              | AFTER FLAME WARP 5X     | SECONDS  | 0        | 0        | 0        | 0        | 0        |
|                              | AFTER GLOW FILL 5X      | SECONDS  | 8        | 9        | 10       | 9        | 5        |
|                              | AFTER GLOW WARP 5X      | SECONDS  | 9        | 9        | 11       | 10       | 6        |
|                              | CHAR LENGTH FILL 5X     | MM       | 14       | 16       | 15       | 8        | 9        |
|                              | CHAR LENGTH WARP 5X     | MM       | 14       | 18       | 15       | 7        | 9        |
|                              | DRIP FILL 5X            | NONE     | 0        | 0        | 0        | 0        | 0        |
|                              | DRIP WARP 5X            | NONE     | 0        | 0        | 0        | 0        | 0        |
| NFPA 1971 8.6                | SHRINK FILL 5MN 500F    | PERCENT  | 0.1      | 0.2      | 0.0      | 0.0      | 0.5      |
|                              | SHRINK WARP 5MN 500F    | PERCENT  | 0.1      | 0.1      | 0.5      | 0.0      | 1.0      |
| NFPA 1971 8.6<br>(AATCC 135) | SHRINK FILL 5MN 500F 5X | PERCENT  | 0.8      | 0.2      | 0.0      | 0.5      | 0.5      |
|                              | SHRINK WARP 5MN 500F 5X | PERCENT  | 0.7      | 0.1      | 0.0      | 0.0      | 0.8      |

## Example No. 2

The following fabrics were also produced and tested. In the following example, both fabrics had a weight of about 6 osy. Sample No. 1

This fabric contained spun yarns and filament yarns in a plain weave. The filament yarns formed a grid-like pattern in the fabric.

Warp Yarn: 21/2 Spun yarn containing 40% polybenzimidazole fibers, 58% para-aramid and 2% Antistat fibers.

The second warp yarn was a 400 denier multi-filament yarn containing para-aramid fibers. The filament yarn accounted for every eighth yarn in the warp direction.

Fill Yarn: 21/2 Spun yarn containing 40% polybenzimidazole fibers, 58% para-aramid and 2% Antistat fibers. The second fill yarn was a 400 denier multi-filament yarn containing para-aramid fibers. The filament yarn accounted for every eighth yarn in the fill direction.

Ends: 44 per inch

Picks: 44 per inch

Weight: 5.80 osy

Weave: Plain weave

## Sample No. 2

The below fabric included spun yarns and filament yarns in both the warp direction and the fill direction. The weave pattern included two spun yarns, one filament yarn, two spun yarns, one filament yarn, etc. in both the fill direction and the warp direction.

Warp Yarn: 30/2 spun yarn containing 49% para-aramid fibers, 49% polybenzimidazole and 2% Antistat fibers.

The filament yarn was a 400 denier filament yarn containing para-aramid fibers.

Fill Yarn: 30/2 spun yarn containing 49% para-aramid fibers, 49% polybenzimidazole and 2% Antistat fibers. The filament yarn was a 400 denier filament yarn containing para-aramid fibers.

Ends: 60 per inch

Picks: 60 per inch

Weight: 5.92 osy

Weave: 2x1 twill weave

| TEST_METHOD          | TEST_NAME           | UNIT        | Sample 1 | Sample 2 |
|----------------------|---------------------|-------------|----------|----------|
| AATCC 118            | OIL REPELLENCY      | AATCC SCALE | 6        | 5        |
| AATCC 135            | SHRINK FILL 5X      | PERCENT     | 0.0      | 0.0      |
|                      | SHRINK WARP 5X      | PERCENT     | 2.5      | 1.0      |
| AATCC 193            | WATER REPELLENCY    | AATCC SCALE | 6        | 6        |
| AATCC 22             | SPRAY RATING        | AATCC SCALE | 100      | 100      |
| AATCC 42             | WATER ABSORPTION    | PERCENT     | 1.0      | 0.4      |
| AATCC 42 (AATCC 135) | WATER ABSORPTION 5X | PERCENT     | 0.5      | 0.0      |
| ASTM D 1777          | THICKNESS           | INCHES      | 0.014    | 0.015    |

| TEST_METHOD               | TEST_NAME               | UNIT     | Sample 1 | Sample 2 |
|---------------------------|-------------------------|----------|----------|----------|
| ASTM D 3774               | WIDTH                   | INCHES   | 59.75    | 61.00    |
| ASTM D 3775               | ENDS                    | THRDS_IN | 44       | 60       |
|                           | PICKS                   | THRDS IN | 44       | 60       |
| ASTM D 3776               | WEIGHT                  | OZ_SQ_YD | 5.80     | 5.92     |
| ASTM D 4032               | CIRCULAR BEND FILL      | POUNDS   | 2.6      | 2.6      |
|                           | CIRCULAR BEND WARP      | POUNDS   | 2.4      | 3.3      |
| ASTM D 5034               | BREAK STRENGTH FILL     | POUNDS   | 256      | 396      |
|                           | BREAK STRENGTH WARP     | POUNDS   | 251      | 394      |
| ASTM D 5034 (AATCC 135)   | BREAK STRENGTH FILL 5X  | POUNDS   | 245      | 468      |
|                           | BREAK STRENGTH WARP 5X  | POUNDS   | 219      | 448      |
| ASTM D 5587               | TRAP TEAR FILL          | POUNDS   | 95       | 292      |
|                           | TRAP TEAR WARP          | POUNDS   | 60       | 314      |
| ASTM D 5587 (AATCC 135)   | TRAP TEAR FILL 5X       | POUNDS   | 54       | 335      |
|                           | TRAP TEAR WARP 5X       | POUNDS   | 52       | 325      |
| ASTM D 6413               | AFTER FLAME FILL        | SECONDS  | 0        | 0        |
|                           | AFTER FLAME WARP        | SECONDS  | 0        | 0        |
|                           | AFTER GLOW FILL         | SECONDS  | 6        | 6        |
|                           | AFTER GLOW WARP         | SECONDS  | 5        | 6        |
|                           | CHAR LENGTH FILL        | MM       | 19       | 14       |
|                           | CHAR LENGTH WARP        | MM       | 23       | 15       |
|                           | DRIP FILL               | NONE     | 0        | 0        |
|                           | DRIP WARP               | NONE     | 0        | 0        |
| ASTM D 6413 (AATCC 135)   | AFTER FLAME FILL 5X     | SECONDS  | 0        | 0        |
|                           | AFTER FLAME WARP 5X     | SECONDS  | 0        | 0        |
|                           | AFTER GLOW FILL 5X      | SECONDS  | 7        | 7        |
|                           | AFTER GLOW WARP 5X      | SECONDS  | 7        | 7        |
|                           | CHAR LENGTH FILL 5X     | MM       | 19       | 13       |
|                           | CHAR LENGTH WARP 5X     | MM       | 17       | 12       |
|                           | DRIP FILL 5X            | NONE     | 0        | 0        |
|                           | DRIP WARP 5X            | NONE     | 0        | 0        |
| NFPA 1971 8.6             | SHRINK FILL 5MN 500F    | PERCENT  | 0.0      | 0.0      |
|                           | SHRINK WARP 5MN 500F    | PERCENT  | 0.7      | 0.0      |
| NFPA 1971 8.6 (AATCC 135) | SHRINK FILL 5MN 500F 5X | PERCENT  | 1.3      | 0.5      |
|                           | SHRINK WARP 5MN 500F 5X | PERCENT  | 1.3      | 0.5      |

These and other modifications and variations to the present invention may be practiced by those of ordinary skill in the art, without departing from the spirit and scope of the present invention, which is more particularly set forth in the appended claims. In addition, it should be understood that aspects of the various embodiments may be interchanged both in whole or in part. Furthermore, those of ordinary skill in the art will appreciate that the foregoing description is by way of example only, and is not intended to limit the invention so further described in such appended claims.

What is claimed:

1. A flame resistant garment comprising:  
a fabric shaped to cover at least a portion of a wearer's body, the fabric comprising first yarns combined with second yarns, the first yarns comprising filament yarns comprised of an inherently flame resistant material, the second yarns comprising spun yarns containing inherently flame resistant fibers, the first yarns being present in the fabric in relation to the second yarns in a ratio greater than 1:1 to less than 1:5, and wherein the fabric includes a warp direction and a fill direction and wherein the first yarns are positioned in both the warp direction and the fill direction and wherein the second yarns are also positioned in both the fill direction and the warp direction.
2. A flame resistant garment as defined in claim 1, wherein the garment comprises a fireman turnout coat and the fabric comprises an outer shell of the garment.
3. A flame resistant garment as defined in claim 1, wherein the first yarns and the second yarns are positioned in the warp direction in a ratio of from greater than 1:1 to about 1:4 and wherein the first yarns and the second yarns are also positioned in the fill direction in a ratio of from greater than 1:1 to about 1:4.
4. A flame resistant garment as defined in claim 1, wherein the first yarns and the second yarns are present in the fabric at a ratio of 1:2.
5. A flame resistant garment as defined in claim 3, wherein the first yarns and the second yarns are present in the fabric at a ratio of 1:2.
6. A flame resistant garment as defined in claim 1, wherein the fibers present in the spun yarns are comprised of a para-aramid.
7. A flame resistant garment as defined in claim 1, wherein the second yarns contain polybenzimidazole fibers.
8. A flame resistant garment as defined in claim 7, wherein the second yarns contain polybenzimidazole fibers in an amount from about 30% to about 60% by weight.
9. A flame resistant garment as defined in claim 1, wherein the fabric has a twill weave.
10. A flame resistant garment as defined in claim 1, wherein the fabric contains polybenzimidazole fibers in an amount from about 20% to about 70% by weight.
11. A flame resistant garment as defined in claim 1, wherein the first yarns have a bigger size than the second yarns.
12. A flame resistant garment as defined in claim 1, wherein the first yarns have a denier of about 600 and the spun yarns have a yarn size of about 18/2 or smaller.
13. A flame resistant garment as defined in claim 1, wherein the first yarns have a denier of about 400 and the spun yarns have a yarn size of about 27/2 or smaller.
14. A flame resistant garment as defined in claim 1, wherein the first yarns have a denier of about 200 and the spun yarns have a yarn size of about 54/2 or smaller.
15. A flame resistant garment as defined in claim 1, wherein the fabric has a basis weight of from about 4 osy to about 9 osy.

**15**

16. A flame resistant garment as defined in claim **15**, wherein the fabric has a circular bend in either a warp direction or in a fill direction of from about 2 lbs. to about 5 lbs. when tested according to ASTM Test D4032.

17. A flame resistant garment as defined in claim **15**, wherein the fabric has a break strength in a fill direction of from about 600 lbs. to about 800 lbs. when tested according to ASTM Test D5034.

18. A flame resistant garment as defined in claim **15**, wherein the fabric has a trap tear in a warp direction of from about 300 lbs. to about 450 lbs. and has a trap tear in a fill direction of from about 250 lbs. to about 400 lbs. when tested according to ASTM Test D5587.

19. A flame resistant garment as defined in claim **15**, wherein the fabric exhibits a char length in a warp direction and in a fill direction of less than about 10 mm when tested according to ASTM Test D6413.

20. A flame resistant garment as defined in claim **3**, wherein the fabric has a basis weight of from about 5 osy to about 8 osy, the first yarns have a bigger size than the second yarns,

**16**

the fabric has a circular bend in either a warp direction or in a fill direction of from about 2 lbs. to about 5 lbs. when tested according to ASTM Test D4032, the fabric has a break strength in a fill direction of from about 600 lbs. to about 800 lbs. when tested according to ASTM Test D5034, the fabric has a trap tear in a warp direction of from about 300 lbs. to about 450 lbs. and has a trap tear in a fill direction of from about 250 lbs. to about 400 lbs. when tested according to ASTM Test D5587 and the fabric exhibits a char length in a warp direction and in a fill direction of less than about 10 mm when tested according to ASTM Test D6413.

21. A flame resistant garment as defined in claim **1**, wherein the fabric has a break strength in a fill direction or in a warp direction of greater than about 60 lbs. per osy.

22. A flame resistant garment as defined in claim **1**, wherein the filament yarns are comprised of a para-aramid, the spun yarns comprising polybenzimidazole fibers combined with aramid fibers, the ratio between the filament yarns and the spun yarns being from about 2:3 to about 1:3.

\* \* \* \* \*